

Dec. 27, 1932.

B. E. ELDRED ET AL

1,892,044

METHOD OF CASTING INGOTS

Filed April 9, 1931



INVENTORS

Byron E. Eldred  
Homer Clyde Snook

George C. Mean

ATTORNEY

# UNITED STATES PATENT OFFICE

BYRON E. ELDRED, OF NEW YORK, N. Y., AND HOMER CLYDE SNOOK, OF SUMMIT,  
NEW JERSEY; SAID ELDRED ASSIGNOR TO SAID SNOOK

## METHOD OF CASTING INGOTS

Application filed April 9, 1931. Serial No. 528,762.

Our present invention involves a solution of the many complicated problems involved in casting ingots of steel and has for its object the production of sound steel ingots suitable for rolling and mechanical working. There are many kinds of steel and steel alloys having widely varying percentage of carbon as well as varying percentages of other ingredients, some beneficial and others detrimental, but our present invention does not particularly concern the composition or the methods of making the various kinds of steel. We assume that the steel will be made in accordance with the best known practices of the art and will be available and ready for pouring; also that in the practice of our method, the pouring ladles and methods, as well as the molds and technique of assembling, lining, luting, etc., will be in accordance with approved practices in these branches of the art.

While our method will be of advantage in connection with any variety of steel, we have preferred to assume for purposes of our present disclosure that the steel is one of the conventional types containing less than  $\frac{1}{2}\%$  of carbon and of good quality as concerns detrimental impurities.

In view of and to a large extent because of the unique qualities of steel, the art of casting has developed along what we find to be entirely improper lines, resulting in serious defects which it is an object of our invention to avoid.

For instance, in the prior art of casting steel ingots, it has been the usual practice to employ cast iron molds whereby the heat is extracted from the molten metal mainly by radial conduction, from the molten interior, outward through the side walls of the iron mold. This has been true for ingots both of the billet and slab types and regardless of whether cast horizontally, vertically or centrifugally. One of the defects, particularly in the case of large ingots intended for roll-

ing and mechanical working, is the formation of blow holes which may be formed either throughout the casting, or near the surface only.

Other defects are piping and/or adjacent segregation of constituents which should be uniformly distributed throughout the ingot. These defects are always serious, due to the waste that results from chopping off a substantial part of the top of each ingot, the top being the part where piping and segregation defects are more or less localized, even where the casting methods are in accordance with the best practices of the prior art.

As set forth in a prior patent to one of us, No. 1,217,581, it has long been recognized that sound castings of copper and other metals having similar qualities of relatively low melting point and high heat conductivity, could be made by a process which "comprises basally and positively cooling a body of molten copper in a thermally conductive mold while exposing the body of the mold to heat, such cooling and heating being so performed as to cause the regular progress upward of the solidification of the molten metal"; also that one method of utilizing the above basic principle is to place a body of such metal in a mold in a flame-heated furnace until the metal melts and then positively cooling the bottom of such mold by placing it on a water cooled floor until the metal solidifies "while still allowing the flame to heat the top of the mold"; also molten copper may be used instead of melting it in the mold. The patent also specifies metals of the same class as including gold, which has practically the same melting point and cooling rate as copper; silver which has slightly lower melting point and higher cooling rate; and aluminum which has a much lower melting point and high cooling rate. The principle is also applicable to zinc which has a much lower melting point but lower cooling rate; also to magnesium, having approximately the same melting point

as aluminum and a cooling rate higher than that of zinc.

We have long recognized that the patented method would be of advantage if it could be applied to making of steel ingots, but the totally different and wholly unique qualities of steel presented difficulties which have heretofore seemed unsolvable.

One difficulty is that steel has a melting point of approximately 1530° C., as against 1080° for copper, or 660° for aluminum, or 650° for magnesium, or 420° for zinc.

On the other hand, the heat conductivity and resulting rate of cooling is far less for steel. While the conduction cooling rates vary somewhat with the temperature and while that of steel is less for those of greater carbon content, the relative cooling rates may be represented in a general way and not too accurately as steel 1, copper 9, aluminum 5, zinc 2.6 and magnesium 3.7. Alloys such as aluminum-bronze are in the same general class as concerns having low melting points and high heat conductivity, as compared with steel.

A vitally important distinction is that steel exhibits the phenomenon of an intermediate state between solid and liquid which is variously described as "mushy", "viscous", etc., and our invention recognizes the problem presented by a body of such relatively non-fluid metal blanketing the solidification surface and tending to prevent escape of gases, slag, etc., which are ejected by the solid at the instant of final solidification.

Our present method for solving the above problems involves abandoning attempts to apply exterior heat to the mold, either for melting solid metal therein or for keeping hot, metal that has been pre-melted and poured into the mold. By our method, the steel is initially super-molten, that is, heated to a temperature as high or higher than that characteristic of what is known as "rising" steel and we utilize the thus stored heat in the molten metal to maintain complete liquidity as against all possible radial heat losses through the top and side walls of the mold, such loss being prevented by heavily insulating the interior of the mold throughout its entire length. Complete liquidity of the contents of the mold being assured for a reasonable time, substantially all of the heat is withdrawn through a water cooled base of the mold. By such method, radial heat losses are made negligible and substantially all of the heat flow is downward parallel with the axis of the ingot. Solidification begins at the bottom and progresses upward substantially at a horizontal plane, thus accomplishing with steel what has been previously accomplished for metals of lower melting point and higher heat conductivity, by the totally different method described in said prior patent. To accomplish this with steel gives a

result not found in the case of copper, namely, the super-molten metal source of heat affords high temperatures, maintaining complete fluidity almost down to the horizontal solidification surface, thereby minimizing the depth of the "mushy" or "viscous" layer, thereby practically eliminating all difficulty of escape of the gas or slag which is ejected from the solidifying surface.

The above and other features of our invention will be more evident from the following description in connection with the accompanying drawing, in which

The figure is a somewhat diagrammatic representation of a mold in which super-molten steel is being solidified in accordance with our present invention.

In this drawing the exterior shell 1 may be of cast iron formed with lifting lugs after the manner of the usual mold, but it is provided with inturned flanges 3 to support a refractory lining the interior surface of which constitutes the mold. The refractory lining preferably comprises a layer of fire brick 4

laid with refractory cement 5. The inner surface of the fire brick lining may constitute the mold but fire brick, though of most excellent non-conducting qualities, are liable to contaminate the steel under certain conditions, and we prefer to employ a thin inner lining 6, which may consist of refractory chromite material which, though slightly more conducting, is likely to be more resistant as concerns contaminating the molten steel. It may be in the form of slabs secured by chromite cement, as shown; or the cement alone may be used. In either case, the entire lining is permitted to dry thoroughly before use. Also it may be initially heated to very high temperature after the manner of refractory lined ladles into which molten steel is drawn for pouring. Moreover, if the steel happens to be of a quality or made under conditions where it is likely to be deficient in super heat, such pre-heating of the lining may immediately precede the pouring of the steel into the mold.

The bottom of the mold is formed by the massive plate 7 supported by and preferably integral with the base 8. This base is preferably formed with a water chamber 9, directly below the plate 7, which chamber is kept cold by circulation of water or other cooling medium through pipes 10 and 11, supplied from any suitable source.

The mold is preferably provided with a "hot top" which may comprise a cast iron shell 12 filled with fire brick 13 and provided with a vent 14 for escape of gases during cooling.

The brick may be of the same thickness as the wall lining brick 4 and the hot top may be dried and may be heated to incandescence just prior to use, as in the case of the mold walls.

The walls of the mold cavity preferably diverge toward the bottom. This facilitates stripping of the ingot and affords and may be specifically designed with a view to progressively smaller cross-sections of molten metal from which the heat is to be drained downward through the base. For instance, if the diameters were top 10" and base 12", the area would be nearly 50% greater at the 10 base than at the top.

Within the mold, we have endeavored to show the solidifying operation, but such showing must be taken as purely diagrammatic. The solidified steel A is indicated as having a vertical grain parallel with the lines of vertical heat flow and perpendicular to the horizontal surface B where the solidification is taking place. C is intended to indicate the thin transition zone where the steel is in the 15 mushy or viscous transition state, and D is intended to represent the great body of super-molten metal which contains heat enough to insure complete liquidity almost down to the 20 surface of solidification at B, thereby making the transition layer C very thin. E is intended to represent the slag on top of the 25 molten steel.

In practice of the invention, the super-molten steel is prepared and poured into the 30 mold according to approved practice in the art, the mold being preheated or not as seems necessary or desirable in any particular case. A sheet of iron or steel may be placed on 35 mold bottom 7 to prevent erosion, if desired.

The water which is kept flowing through the water chamber 9, in cast iron base 8, extracts heat from the bottom 7 which in turn extracts heat rapidly from the bottom of the 40 liquid steel. By extracting the heat from the liquid steel rapidly and from the lower end of the ingot only, a number of beneficial results are obtained in the resulting solidified metal, A. The solidification progresses in 45 an upwardly shifting horizontal plane, and the crystal formation grows from the bottom upward with the major axes of the crystals vertical to said plane and parallel with the length of the ingot, as diagrammatically indicated. The crystal axes are thus parallel 50 with each other and parallel with the direction of extension of the metal when subsequently rolled. They are thus in the most favorable position to afford maximum ductility, density and strength for the rolled 55 product.

Heretofore the best and strongest metal has been found in the lower portions of ingots 60 that have been cast in wall-chill molds. In such case the lower portions of the ingot are solidified in basaltic columns and are cleaner and stronger than the metal in the rest of the 65 ingot. By our method, the steel is solidified rapidly upwards so that basaltic columns of strong, equiaxed crystals, extend longitudi-

nally throughout the ingot, instead of being confined to the bottom of the ingot.

This may be explained on the theory that gases and slag dissolved in steel are rejected by it at the instant of freezing and by our process the steel freezes upward uniformly so that a substantially horizontal boundary is maintained between the solid steel and the fluid steel. Moreover, all of the layer or layers of intermediate transition temperatures, 70 where the steel passes through the more or less viscous plastic states, are also horizontal and of uniform vertical thickness. Hence they offer uniform, minimum resistance to uniform vertical upflow of gas and slag ejected from the freezing surface. Because this surface is substantially horizontal and such flow lines are vertically upward, while heat abstraction is vertically downward, the crystals grow vertically upward. 75

Hence, the gas and slag are correlative more free to escape upward between such vertical crystals, instead of being trapped by horizontal crystals such as grow from the side walls of the mold when the ingot is 80 frozen by side wall cooling processes heretofore employed. In this connection, it is to be noted that in the prior art, cooling of the steel, even when applied to the side walls progressively, from the lower portions upward, has not been controlled by effective side wall insulation, and the result has been that side wall freezing has progressed in advance of interior freezing, thus causing the crystals 85 to grow and the viscous zones to develop radially, instead of vertically throughout a large part of the ingot volume, thereby causing entrapment of gas, piping, liquation, segregation and coarse crystallization. It is obvious that under such conditions a large part 90 of the metal is being cooled all the time, and even though this may result in a shorter total time for the final cooling, the actual cooling time at any one point is relatively long. The point is that the longer the cooling time of any given zone or layer independently of the total cooling time, the more voluminous will 95 be the viscous zone, the coarser the crystallization on freezing, the greater the segregation, the greater the liquation, and the greater 100 the tendency to pipe formation. 105

By our method, the body of liquid is initially super-molten and the complete side wall insulation keeps this liquid from cooling to mushy temperatures except as and where heat is conducted downward through the horizontal freezing surface. Under such conditions, by extracting the heat rapidly by water cooling at the lower end of the ingot, while rendering side wall cooling practically negligible, we are able to reduce the size of the crystals and to prevent or minimize liquation and segregation, and to prevent the formation of pipes. 110

Naturally, the hotter the mass of liquid 115

steel when poured into the mold and the more rapidly the heat is extracted from the bottom of the ingot, the thinner will the viscous layer be squeezed, so to speak, between the 5 hot molten metal and the advancing surface of the freezing, solid steel.

This viscous layer being thin, the fraction of the volume of the ingot in the viscous state at any one time is small, and the time between 10 liquid and solid state is small. Hence our method involves quick freezing and smaller crystals and such segregation and liquation as can take place is very small in amount because the volume of viscous metal upon 15 which crystals can feed is small and the time is short.

Thus, by our method of orderly, localized, rapid heat extraction from the molten steel, we produce in the solidified ingot a crystalline structure that, in addition to being dense, ductile and homogeneous, is made up of small-sized, equiaxed crystals. Consequently, our ingots require less mechanical working and rolling to yield the desired fine 25 grained, homogeneous structure required in a strong and tough finished product.

It is understood that the steel to be cast by our process should be deoxidized and degassed before pouring as well as is practicable, considering the present state of the 30 art. The proper use of a sufficient quantity of aluminum, ferro-silicon or other well known deoxidizers may be desirable.

While the great, outstanding merit of our 35 present invention, is its successful application to and solution of the unique problems of steel ingot casting, it will be evident that it is applicable to other metals or alloys of far lower melting point and higher conductivity, 40 as well as to those of high melting point and of either higher or lower conductivity than steel.

We claim:

1. In the art of casting an elongated steel 45 ingot to be further elongated by rolling or the like, a process which includes forming an elongated upright mold of insulating material constituting the lining of an exterior cast iron casing mold; charging said mold with liquid steel hot enough to insure initial super-molten 50 temperature for all of said liquid and for the top and side walls of said insulating liner mold; cooling the lower end of the liquid so as to form a solid layer having a substantially horizontal top; and thereafter causing solidification to progress upward in a substantially horizontal plane by abstracting heat from the liquid downwardly and substantially uniformly throughout all 55 parts of the pre-formed surface.

2. In the art of casting an elongated steel ingot to be further elongated by rolling or the like, a process which includes forming an elongated upright mold of insulating material 60 constituting the lining of an exterior cast iron

casing mold; charging said mold with liquid steel hot enough to insure initial super-molten temperature for all of said liquid and for the top and side walls of said insulating liner mold; chilling the bottom of the mold; the 70 heat insulation afforded by the sides and top of the mold being sufficient to cause the bottom chilling to effect solidification of the steel in an upwardly creeping approximately horizontal boundary between the solid and the 75 liquid.

3. In the art of casting an elongated steel ingot to be further elongated by rolling or the like, a process which includes forming an elongated upright mold of insulating material 80 constituting the lining of an exterior cast iron casing mold; charging said mold with liquid steel hot enough to insure initial super-molten temperature for all of said liquid and for the top and side walls of said insulating liner mold; and chilling the steel by removing heat 85 congelations from a narrow horizontal zone by downflow of the heat substantially uniformly through all of the top area of the pre-formed solidified material.

4. In the art of casting an elongated steel ingot to be further elongated by rolling or the like, a process which includes forming an elongated upright mold of insulating material 90 constituting the lining of an exterior cast iron casing mold; charging said mold with liquid steel hot enough to insure initial super-molten temperature for all of said liquid and for the top and side walls of said insulating liner mold; and chilling the steel by removing heat 95 congelations from a narrow horizontal zone by downflow of the heat substantially uniformly through all of the top area of the pre-formed solidified material.

5. A method of casting ingots having a grain structure of the metal disposed approximately parallel with the direction in which the metal is to be elongated, which method includes charging the metal super-molten, 100 heat insulating its interior, metal contacting surface to substantially prevent solidification by cooling at one end and also by cooling transversely of the desired direction of the grain, solidifying the other end by withdrawing heat from the liquid substantially uniformly over all the area of said other end, and thereafter similarly, uniformly and progressively withdrawing substantially all of the heat through the advancing pre-formed 105 surface of the solid.

6. A method of casting elongated ingots having a grain structure disposed approximately parallel with the axis of the ingot, which method includes charging the metal, 110 super-molten, into an upright mold; heat insulating its interior, metal containing surface to substantially prevent solidification by cooling horizontally or through the top; solidifying a horizontal layer at the bottom by 115 withdrawing heat from the liquid down- 120

wardly and substantially uniformly through all portions of the area of said bottom; and thereafter progressively solidifying the remaining liquid by withdrawing substantially 5 all of the liquefying heat downwardly and substantially uniformly through all portions of the area of the advancing pre-formed surface of the solid.

Signed, at New York, in the county of 10 New York and State of New York, this 8th day of April, A. D. 1931.

BYRON E. ELDRED.  
HOMER CLYDE SNOOK.

15

20

25

30

35

40

45

50

55

60